

## UNITED STATES PATENT OFFICE.

CHARLES C. RUPRECHT, OF OLMSTED, ILLINOIS.

## PROCESS OF PREPARING FULLER'S EARTH.

No Drawing.

Application filed January 8, 1921. Serial No. 435,945.

*To all whom it may concern:*

Be it known that I, CHARLES C. RUPRECHT, a citizen of the United States, residing at Olmsted, in the county of Pulaski and State 5 of Illinois, have invented a certain new and useful Improvement in Processes of Preparing Fuller's Earth, of which the following is a full, clear, and exact description.

This invention relates to a process for the 10 preparation of fuller's earth, with the view of increasing the efficiency thereof in accordance with the particular materials with which such earth is to be used.

As is well known, the peculiar property 15 possessed by fuller's earth of removing colors from oil or other solutions is believed to be due to an absorption (through the pores or cells of such earth) of the coloring matter—the action being mechanical and not 20 chemical.

It has been found that fuller's earth from different localities varies in its action upon liquids, some earths giving better results with a particular oil or material than with 25 another oil or material and different earths giving different results with the same oil or material. This has resulted in a selection, for a particular oil or material under treatment, of the grade of earth that has been 30 found by experience to be best adapted therefor.

An examination of the different fuller's earths discloses the fact that such earths are 35 of a highly porous nature, being made up of tubular cells consisting mainly of hydrous aluminum silicate. The cells contained in any particular kind of fuller's earth are of practically uniform size and shape, but they differ in size and shape in different earths 40 or earths from different localities. Earths from one locality or deposit may contain cells of one particular shape and internal diameter while earths from other localities or deposits may and do contain cells of 45 different shapes and diameters; and it is believed that this difference in the shapes and the internal diameters of the cells accounts for the different in the action of the various fuller's earths upon oils and other materials.

50 In an endeavor to secure a uniform and efficient action from fuller's earth, it has been the practice to reduce the same to a dry condition and then grind it to a fineness depending upon the use to which it is to be put. For the treatment of mineral oil, the 55 earth is reduced to a fineness of 15-30 mesh,

30-60 mesh, and 60-90 mesh according to the particular oil to be treated; while, for edible oils, the earth is frequently reduced to a fineness of 200 mesh. In drying the 60 earth, the practice has been to heat it until all of the hygroscopic water has been driven off and most of the combined water liberated, using for this purpose a temperature of at least 900 degrees F. This method of 65 treatment has resulted in ruining many good clays and has proven detrimental in a great many cases, due to the excessive heating.

I have found that the entanglement of the 70 coloring matter of oil or other materials under treatment in the pores or cells of fuller's earth depends on three factors, namely; the size and shape of the pores or cells in the earth, the dimensions of the 75 coloring material (which may be in a colloidal condition), and the surface conditions of the pores or cells. By the modes of treatment set forth hereinafter, I have been enabled to produce the proper conditions in the cells or pores of the earth to enable the 80 latter to operate efficiently with any particular medium under treatment.

In some fuller's earth of low grade, the 85 pores or cells have been found to be of such large size and the capillary and colloidal action of the same to be of such low intensity as to enable the retention of only a small portion of the coloring matter contained in the medium being treated. In still other 90 earths, the pores or cells are so small as to entangle only the smallest particles of the coloring matter, resulting in a clogging of the earth and a decrease in its decolorizing power and efficiency.

Where the pores or cells are of greater 95 cross sectional area than is desirable, I subject the earth to either of the two following treatments:—

(A) I take advantage of the shrinkage 100 characteristics of the earth in the following manner. In the process of manufacture and use, it is slowly and uniformly heated until most of the hygroscopic water is driven off. The shrinkage taking place gradually and at a temperature not much in excess of 400 degrees F. In continuation of the process, the earth is subjected to a temperature greatly in excess of the former temperature for a period sufficient to give a "set" or surface 105 hardening thereto which tends to maintain 110 the internal structure of the earth against attrition. For the purpose of securing this

"set" or surface hardening, it is usually sufficient to pass the earth through an open flame and to retain it therein for a few minutes, at most. In some cases, as where the earth is desired for high grade oils, the final heating and tempering or setting will be realized by the use of heated members and without subjecting it directly to gases of combustion.

10 By the treatment described, the earth is uniformly and gradually shrunk until the proper area of cells or pores is secured, being set in this condition through the sudden application of a higher temperature to its 15 surface.

(B) As a modification of the manner of reducing the pore or cell area above described, the earth will be first dried to an extent necessary to free it from most of the 20 hygroscopic water, after which it will be percolated or saturated with a solution containing an organic or inorganic colloid, such as albumin, glue, or the mineral colloids. The earth will then be freed from most of the 25 solution by percolation or other means and then dried, as in a rotary kiln. In the drying operation, the earth may be raised to a temperature sufficient to secure carbonization of the colloidal material remaining 30 in the pores; but this will not usually be necessary unless the material is very dense.

While I have referred to the use of colloidal material for reducing the cross sectional area of the cells or pores and prefer 35 this mode of reduction, I do not intend to be limited to the use of such material, as other materials may be employed, provided that they are capable of depositing upon the walls of the pores or cells a layer that will 40 reduce the cross sectional area thereof but without entirely or unnecessarily obstructing the same. For instance, the earth may be saturated with coal gas and then heated sufficiently to break down the gas and de- 45 posit carbon within the pores, the heating operation being carried on in an atmosphere limited as to oxygen to render imperfect the combustion of such gas.

In some cases, a material that will act as a 50 mordant may be employed for the purpose of reducing the cross sectional areas of the cells or pores. Instances of such mordants are stannic solutions—as a chloride, a chromate, or a sulphate of tin; also salts of 55 alumina and silicic acid—the action depend-

ing upon the colloidal deposition of such material.

Where the pores or cells are of smaller cross section area than is desirable, I may enlarge the same as follows. The earth under treatment is subjected to the action of a solvent for the mineral matter, instances of such solvent being a solution of sodium hydrate or sodium carbonate, or of an acid, the solvent being capable of acting upon the 65 silicates or other mineral matter of the earth. The solution is allowed to act upon the earth under treatment for a sufficient time to secure the proper enlargement of the pores or cells, after which it is neutralized, as by washing or by other suitable means, and the earth then dried and prepared in the ordinary manner. An acid solvent that may be used to advantage is carbonic acid gas dissolved in water, the particular reagent not only enlarging the pores themselves but leaving the surfaces of the same in an active colloidal condition.

While my invention has been described as specially adapted for the preparation of fuller's earth it will be applicable to other clays, as I have found it possible through the mode of treatment described herein to impart a degree of decolorizing action to clays that previously did not possess such capability. Hence, by the use of the expression "fuller's earth" in the claims, I do not propose to limit my invention to the particular clays now known to the trade as fuller's earth.

Having thus described my invention, what I claim is:

1. The process of preparing fuller's earth which comprises drying the same to free it from hygroscopic water contained therein, 95 saturating the earth thus treated with a colloidal solution, removing from the pores or cells a proportion of such solution, and drying the earth.

2. The process of preparing fuller's earth which comprises removing hygroscopic water therefrom, then treating the earth with a reagent capable of leaving within the pores or cells thereof surfaces of colloidal material, and drying the earth thus treated.

In testimony whereof, I hereunto affix my signature.

CHARLES C. RUPRECHT.